# EUROPEAN PATENT APPLICATION

(11) **EP 0 535 608 A1**
(43) Date of publication of application: **07.04.1993**
(21) Application number: 92116677.3
(22) Date of filing: 29.09.1992
(51) Int. Cl.: B41M 5/38

(54) **Thermal-transfer material and the image-forming process using the same material**

(30) Priority: 04.10.1991 JP 258005/91
(71) Applicant: KONICA CORPORATION, Tokyo 163 (JP)
(72) Inventor: Komamura, Tawara, KONICA CORPORATION, Hino-shi, Tokyo (JP); Miura, Norio, KONICA CORPORATION, Hino-shi, Tokyo (JP); Nakayama, Noritaka, KONICA CORPORATION, Hino-shi, Tokyo (JP); Tanaka, Tatsuo, KONICA CORPORATION, Hino-shi, Tokyo (JP); Nakayama, Yoriko, KONICA CORPORATION, Hino-shi, Tokyo (JP)
(74) Representative: Henkel, Feiler, Hänzel & Partner

(57) **Abstract**

A thermal-transfer material having a dye containing a phenolic hydroxy group, or a 3-coordinated chelatable dye, is disclosed. When making use of the materials, a color image having an excellent hue and a high density can be obtained. And the effects of the fixability can be more than in the case where a mordant is contained in an image-receiving material.

## Description

### Field of the Invention

This invention relates to a thermal-transfer material and the image forming process in which the thermal-transfer material is used and, particularly, to the thermal-transfer material having a high sensitivity and an excellent preservability and the image forming process in which the thermal-transfer material is used.

### Background of the Invention

As for the processes for obtaining an image in a simple and dry treatment and, particularly, for obtaining a high-quality full-color image, there are the processes in which a thermal-transfer material is used. In the thermal-transfer materials, the dyes to be used for forming a color image are particularly important and, therefore, various kinds of dyes to be used for thermal-transfer materials have been proposed. For example, Japanese Patent Publication Open to Public Inspection (hereinafter referred to as JP OPI Publication) Nos. 3-83686/1991, 3-83687/1991, 3-83688/1991, 3-83689/1991, 3-114890/1991, 1-228601/1989, 1-229755/1989, 1-229756/1989 and so forth have proposed the processes for forming an image, wherein a dye having a phenolic hydroxyl group is so used as to make a reaction with a mordant contained in an image-receiving layer and the image is formed by the dye produced by the reaction.

When the dye and the mordant are completely reacted, the image formed by the dyes described in the above-given patents have the excellent characteristics capable of improving the problems raised by the conventional thermal-transfer, such as a satisfactory hue and an excellentfixability. However, in a thermal-transfer image formation, there may be some instances where the unfavorable problems such as the presence of an irregular absorption or a fixability failure may be produced due to the dichroism caused by an unreacted dye residue without fully completion of the reaction, because the image formation is carried out in an extremely short time by applying heat from a thermal head. In addition, JP OPI Publication Nos. 59-78893/1984, 59-109394/1984 and 60-2398/1985 disclose the image forming processes for forming an image on an image-receiving material by using a chelated dye.

The above-mentioned image forming processes are excellent as the processes for improving a fixability and, at the same time, for improving an image stability such as a light fastness. However, still in the image forming processes disclosed in the above-given patents, there have been the defects such as a colorcontam- ination and a fixability failure produced by an unchelated dye residue, because the chelation is not fully performed in a transfer.

For improving a transferability, U.S. Patent No. 4,876,236 and JP OPI Publication Nos. 1-113275/1989, 1-332952/1989. 2-1386/1990, 2-1387/1990, 2-57322/1990, 62-111784/1987 and 61-286199/1986 propose that an additive is added to a dye donative layer. However, in these patents, there is no description of the addition of any organic base. It is further unfavorable when an organic base is added to a dye donative layer and transferred to an image-receiving layer, because the light fastness of the transferred image is seriously deteriorated.

Further, in the thermal-transfer materials including, particularly, the so-called sublimation type thermal-transfer materials, there are not only the problems in an image fixability, but also the problems in the preservability of the thermal-transfer materials themselves, which are derived from the diffusibility of dyes, because the dyes are thermally diffusible. For example, in the case that preserving a thermal-transfer material in the state where the surface thereof is superposed on the other surface (such as in the rolled form), there is a problem that the dyes are transferred to the other surface. These preservability problems have been solved by making the transferability of the dyes lower, and that has had the defect that the sensitivity of a thermal-transfer material is caused to be lowered thereby.

### Summary of the Invention

It is an object of the invention to improve the above-described problems. To be more concrete, it is an object of the invention to provide a thermal-transfer material high in sensitivity and excellent in preservability. Another object of the invention is to provide a thermal-transfer material capable of a color image satisfactory in hue, high in density and excellent in fixability. And, a further object of the invention is to provide an image forming process in which a thermal-transfer material capable of forming a color image high in density and excellent in image stabilities such as fixability and light fastness.

As the results of the earnest studies made by the present inventors, it was discovered that a thermal-transfer material which was applied with a dye excellent in thermal diffusibility and the salt of a nitrogen-containing organic base is amagingly high in sensitivity and excellent in preservability of the thermal-transfer material. Besides the above, when making use of the salt of a dye and a nitrogen-containing organic base (herein after referred to as a dye salt), it was also discovered to improve the reactivity of the dye with a mordant without lowering the dye-transferability in forming a thermal-transfer image and to improve the problems raised by a dye remaining unreacted with the mordant. Besides the above, when making use of a chelatable dye salt, it was further discovered to improve the reactivity with a metal ion-donative compound (hereinafter referred to as a metal source) without lowering the dye transferability in forming a thermal-transfer image and to improve the problem raised by a dye remaining unreacted with a metal source. From the above-mentioned discoveries, the invention have been completed.

The above-mentioned objects of the invention can be achieved with a thermal-transfer material comprising a support having a layer containing a dye thereon, wherein; a dye forms a salt with nitrogen-containing organic base; in an image forming process, comprising using a thermal-transfer material, bringing a dye salt-containing thermal-transfer material into close contact with an image-receiving material having a mordant-containing image-receiving layer, and forming an image in the image-receiving layer of the image-receiving material upon applying heat thereto according to an image information; and in an image forming process comprising using a thermal-transfer material, bringing the thermal-transfer material containing the salt of a chelatable dye and a nitrogen-containing organic base (hereinafter referred to as a chelatable dye salt) into close contact with an image-receiving material having an image-receiving layer in the presence of a metal source, applying heat thereto and forming an image in the image-receiving layer according to an image information.

### Brief Description of the Drawings

Fig. 1 : An illustration of an example of the image forming processes comprising using a thermal-transfer material of the invention; and
Fig. 2 : An illustration of another example of the image forming processes comprising using another thermal-transfer material of the invention;
   wherein
   1 : Support for an image-receiving material;
   2 : Image-receiving layer;
   3: Image-receiving material;
   4 : Support for a thermal-transfer material;
   5 : Thermal-transfer layer;
   6, 10 : Thermal-transfer materials;
   7 : Thermal head;
   8 : Exothermic resistor;
   9 : Thermofusible layer;
   9a: Cohesion broken down- or interface peeled off-thermofusible layer;
   11 : Plain paper image-receiving material

### Detailed Description of the Invention

There is no special limitation to the dyes capable of forming the dye salts of the invention, provided that they are able to form a saitwith a nitrogen-containing organic base. The dyes conventionally applicable to thermal-transfer materials including, for example, an azo dye, an azomethine dye and an anthraquinone dye (such as the dyes and the derivatives thereof each given in Kinki Chemical Society, 'Data from the Sectional Committee of Functional Dyes', No.16, pp.34-35. Among the dyes, the drivatives having a phenolic hydroxyl group are particularly desirable from the viewpoints mentioned later.)

Among these dyes, a dye having a phenolic hydroxyl group is desirably be used for forming a nitrogen-containing organic base and a salt with keeping a high sensitivity (that is the high transferability of a dye). Also, in the case where an image is formed by using a mordant, the dyes having a phenolic hydroxyl group are desirably used from the viewpoint of making the high transferability and the mordantability compatible. The dyes having such a phenolic hydroxyl group as mentioned above include, for example, the derivatives having a phenolic hydroxyl group of the above-mentioned dyes and those given in JP OPI Publication Nos. 3-83686/1991, 3-83687/1991, 3-83689/1991, 30114890/1991, 3-90387/1991, 3-90387/1991, 3-92385/1991 and 3-92386/1991.

The particularly desirable dyes having a phenolic hydroxyl group include those represented by Formula (I).
[wherein R represents a group forming an azomethine dye together with =N-C₆H₄-OH, provided, the benzene ring may also have a substituent].

The concrete examples thereof include those given in JP OPI Publication Nos. 3-83687/1991, 3-83688/1991, 3-83689/1991, 3-114890/1991, 3-90387/1991, 3-92385/1991 and 3-92386. The typically concrete examples of the dyes having Formula (I) will be given below.

Next, the chelatable dyes (hereinafter referred to as chelatable dyes) will be detailed.

The chelatable dyes each having a hydroxyl group may be used upon suitably selecting from the various kinds of well-known compounds. For example, they include the cyan-image forming dyes (hereinafter referred simply to as cyan dyes), the magenta-image forming dyes (hereinafter referred simply to as magenta dyes) and the yellow-image forming dyes (hereinafter referred simply to as yellow dyes) each given in JP OPI Publication Nos. 59-78893/1984 and 60-2398/1985 and JP Application Nos. 2-213303/1990, 2-214719/1990 and 2-203742/1990.

Among them, a dye capable of forming at least the foregoing metal ion-containing compound and three chelates may desirably be used. In particular, a three coordinated chelate dye having a phenolic hydroxyl group may particularly be desired to use from the viewpoints for forming a dye salt with keeping a high sensitivity and improving excellent color tone and light fastness. The particularly desirable chelate dyes are those represented by Formula (II).

[wherein A represents an aryl group or a heterocyclic group and at least one of the adjacent positions of carbon atom bonding to the azo bond of the aryl or heterocyclic group is a carbon atom substituted with a chelatable hetero atom or a chelatable group; and Z represents the group consisting of atoms necessary to form a 5- or 6-member ring.]

The nitrogen-containing organic bases capable of forming a dye salt include, desirably, an organic base having a pKa of not less than 9. They include, for example, primary through tertiary alkyl amines (such as octyl amine, dibutyl amine and triethyl amine). The particularly desirable organic bases include the compounds represented by the following Formula (III). These compounds include, for example, amidine, guanidine, guanidine derivatives and the vinyl type derivatives thereof.
wherein R₁, R₂ and R₃ represent each a hydrogen atom or an alkyl group; R₄ represents a hydrogen atom, an alkyl group, an aryl group, an amino group (including an alkyl-substituted amino group) or a guanidine group, provided, R₁ and R₂ and/or R₃ and R₄ may be so coupled to each other as to form a ring; X represents a vinyl group; and n is an integer of 0 or 1.

The typical examples of the bases represented by the above-given Formula (III) include B-1 through B-27 given in JP OPI Publication No. 64-3653/1989, pp.3 - 4.

In addition to the above, the following organic bases are also desirable.

The dye salts of the invention can be prepared by mixing the foregoing dyes and the foregoing organic bases into a suitable solvent (such as ethyl acetate, acetone and ethanol).

In the thermal-transfer materials of the invention, the dye salt content is, desirably, within the range of 0.05 to 10 g per m² of the support used therein.

The dye salt layers of the invention have a binder for maintaining the dye salts.

The binders include desirably, Those made of solvent-soluble polymers such as acryl resin, methacryl resin, polystyrene, polycarbonate, polysulfone, polyether sulfone, polyvinyl butyral, polyvinyl acetal, nitrocellulose and ethyl cellulose. These binders may be used independently or in combination not only by solving them in an organic solvent, but also in the form of a latex-dispersion. The binders may be used desirably in an amount within the range of 0.1 to 20 g per m² of the support used.

The dye salt-containing layers can be formed in the following manner. A thermal-transfer layer-forming ink- solution is prepared either by dissolving the salts of the invention independently or in combination together with a binder in a solvent or by dispersing them in the finely particulate form in a solvent and the resulting ink-solution is coated on a support and is then dried up. The dried thickness of the dye-containing layer is desirably within the range of 0.1 to 10wm.

There is no special limitation to the supports, provided, they are satisfactory in dimensional stability and resistive against any heat application such as a heating made by a thermal head in thermal-recording operation. The supports desirably used for include, for example, a condenser paper, a thin-leaf paper such as glassine paper and a heat-resistive plastic film such as those made of polyethylene terephthalate, polyamide and polycarbonate. The thickness of the support is desirably within the range of 2 to 30µm. The support is also desired to have a sublayer comprising a polymer selected for the purposes of improving the adhesive property to a binder and preventing a dye-transfer and dyeing to the support. Further, a slipping layer may also be provided to the rear surface of the support (i.e., the opposite side to a dye-containing layer) for the purpose of preventing the tacky adhesion of a head to the support.

For applying the thermal-transfer material of the invention to a full-color recordable thermal-transfer material, it is desired to repeatedly coat a yellow thermal-transfer layer containing a salt comprising a yellow dye, a magenta thermal-transfer layer containing a salt comprising a magenta dye and a cyan thermal-transfer layer containing a salt comprising a cyan dye in total of three layers in order on one and the same surface of a support. If required, a thermal-transfer layer containing a black-image forming material, in addition to the above layers totalling 4 layers, may also be repeatedly coated in order on one and the same surface.

In the thermal-transfer recording processes, the dye-containing layer of a thermal-transfer material and the image-receiving layer of an image-receiving material are superposed on each other and heat is applied to the thermal-transfer material so as to meet an image information, so that the image is formed ob the image-receiving material by the dye having formed a salt.

The image-receiving materials of the invention have an image-receiving layer on the support thereof.

As for the supports for the image-receiving materials, paper, plastic films or a paper-plastic film complex may be used. The supports include, concretely, those given in JP OPI Publication No. 3-54556/1991, p.5,17th line in the upper right column - 11th line in the lower left column.

The image-receiving layers are each comprised of a polymer binder. The polymer binders include, desirably, a thermoplastic polymer. The image-receiving layers are comprised of one or not less than two kinds of polymer layers such as those made of polyester resin, polyvinyl chloride resin, a vinyl chloride-the other monomer (such as vinyl acetate) copolymer, polyvinyl butyral, polyvinyl pyrrolidone or polycarbonate.

In the invention, it is desired to contain a mordant in an image-receiving layer. When this is the case, a dye salt and a mordant are each reacted together, so that an image may be fixed.

The mordants include, for example, a compound having an amino group such as those having an alkyl amine (e.g., decanoyl amine, octyl amine, dioctyl amine and trioctyl amine), an aryl amine (e.g., an aniline derivative) and those having a nitrogen-containing heterocyclic group (e.g., a pyridine ring and an imidazole ring).

The mordants are desired to be immobilized and a polymer mordant is particularly desirable. The polymer mordants are described in, for example; JP OPI Publication Nos. 48-28325/1973, 54-74430/1979, 54-124726/1979, 55-22766/1980, 55-142339/1980, 55-23850/1980, 60-23851/1985, 60-23852/1985, 60-23853/1985, 60-57836/1985, 60-60643/1985, 60-118834/1985, 60-60643/1985, 60-118834/1985, 60-122940/1985, 60-122941/1985, 60-122942/1985 and 60-235134/1985; U.S. Patent Nos. 2,484,430, 2,548,564, 3,148,061, 3,148,161, 3,309,690, 3,756,814, 3,898,088, 3,958,995, 4,115,124, 4,124,386, 4,193,800, 4,273,853, 4,282,305 and 4,450,224; and British Patent Nos. 1,594,961, 2,056,101 and 2,093,041.

When the dye salt of the invention comprises a chelatable dye, an image-receiving layer is desired to contain a metal source. The metal sources include desirably the inorganic or organic salts of the metal and the complexes of the metal. The metal ions constituting a metal source include, for example, a divalent or polyvalent metals belonging to the I through VIII Groups of the periodic table. Among them,.Al, Co, Cr, Cu, Fe, Mg, Mn, Mo, Ni, Sn, Ti and Zn are desirable and, particularly, Ni, Cu, Co, Grand Zn are preferable. The typical examples thereof desirably applicable to the metals include the complexes represented by the following formula, in which Ni2⁺, Cu2+, Co2+, Cr²⁺ and Zn²⁺ are contained.
wherein M represents a metal ion; 0₁, Q₂ and Q₃ represent each a coordination compound capable of coordinate-bonding to the metal ion represented by M, provided that they may be selected from the coordination compounds such as those given in'Chelate Chemistry (5)', (Nankoh-Do) and that, in particular, they may desirably include ethylenediamine and the derivatives thereof, glycine amide and the derivatives thereof, picoline amide and the derivatives thereof, or β-diketone and the derivatives thereof, represented by formula
wherein R¹ and R² each represent an alkyl group which may be substituted. L represents an anion capable of forming a counter-anion with a complex, provided that they may include inorganic compound anions such as CI-, S0₄- and ClO₄⁻ and organic compound anions such as a benzenesulfonic acid derivative and an alkylsulfonic acid derivative and that, in particular, they may desirably include a tetraphenyl boron anion and the derivatives thereof; 1 is an integer of 1, or 3; m is 1, or 0; n is 1 or 0; provided, these are determined by whether a complex represented by the foregoing formula has a coordination number of 4 or 6, or by the numbers of the ligands of Qₗ, Q₂ and Q₃; and p is 0, 1, 2 or 3.

A metal source is usually added to an image-receiving material and, desirably added to the image-receiving layer of an image-receiving material or the foregoing thermofusible layer thereof. The metal sources are added in an amount within the range of 0.2 to 20 g/m² of an image-receiving material or a thermofusible layer and, desirably, 1 to 10 g/m² thereof.

In the thermal-transfer recording processes of the invention, the thermal-transfer layer of the above-mentioned thermal-transfer recording material and an image-receiving material are superposed together and heat is then applied to the thermal-transfer recording material so as to meet an image information, so that an image can be formed on the image-receiving material with a chelate dye formed upon reaction of a metal source with a dye of the invention. In the invention, the dyes represented by the foregoing Formula (I) are used for the dyes. Therefore, a magenta image can effectively be obtained so as to have a high density, a rich image stability and desirable color-reproduction. The above-mentioned metal sources may be made present either in an image-receiving material or in a thermofusible layer provided onto a thermal-transfer layer.

The thermal-transfer recording processes of the invention will be detailed with reference to the drawings. In Fig.1, when a metal source is made present in the image-receiving layer of image-receiving material 3 comprising support 1 and image-receiving layer 2, the foregoing dyes contained in the thermal-transfer layer of thermal-transfer material 6 comprising support 4 and thermal-transfer layer 5, such dyes are diffusedly transferred to image-receiving material 3 by applying heat thereto from exothermic resistor 8 of thermal head 7, for example, and the transferred dyes are reacted with a metal source in image-receiving layer 2, so that a chelate dye image can be formed. In Fig.2, when making a metal source present in thermofusible layer 9 provided onto thermal-transfer layer 5, the dyes contained in thermal-transfer layer 5 of thermal-transfer material 10 comprising support 4, thermal-transfer layer 5 and thermofusible layer 9, such dyes are diffusedly transferred to thermofusible layer 9 by applying heat thereto from exothermic resistor 8 of thermal head 7, for example, and the transferred dyes are reacted with a metal source there so as to form a chelate dyes, so that an image can be formed by cohesion-destroying or interface-peeling the thermofusible layer containing the chelate dyes and then by transferring the destroyed or peeled thermofusible layer to image-receiving material 11.

### EXAMPLES

The invention will be concretely detailed with reference to the following examples. It is, however, to be understood that the embodiments of the invention shall not be limited thereto.

### EXAMPLE 1

### (Synthesis of the dye salt of the invention)

(1-3) of 7.6 g and tetramethyl guanidine (TMG) of 2.5 g were mixedly stirred in acetone and the solvent was condensed. The resulting solid was recrystallized with toluene, so that the tetramethyl guanidine salt (S-1) of 1-3, that was the object matter, could be obtained. In the same manner, the dye salts (S-2 through S-1 0) shown in Table 1 could also be obtained.

### (Preparation of an ink)

The following raw materials were mixed up together so as to obtain the ink of a uniform solution containing the dye salt relating to the invention.

### (Preparation of a thermal-transfer material)

The resulting ink was coated on a 4.5µm-thick polyethylene terephthalate base by making use of a wire-bar and then dried so as to have a dried amount coated of 0.8 g/m², so that thermal-transfer material Acorn- prising a thermal-transfer layer formed on a polyethylene terephthalate film. On the rear surface of the film base, a nitrocellulose layer containing silicone-denatured urethane resin (SP-2105 manufactured by Dai-Nichi Seika) was provided as a sticking-preventive layer.

Separate from the above, thermal-transfer materials B through J each having the same constitution as those of thermal-transfer material Awere prepared in the same manner as in thermal-transfer material A, except that dye salt S-1 of thermal-transfer material A was replaced by the dye salt of the invention shown in Table 1.

### (Preparation of an image-receiving material)

On a paper support laminated with polyethylene on the both sides thereof (containing a white pigment (Ti0₂) and a bluish coloring agent), a methylethyl ketone solution containing polyvinyl chloride resin containing ester-denatured silicone (in an amount coated of 0.15 g/m²) was coated for serving as an image-receiving layer so that the amount of the resin coated could be 5 g/m², thereby image-receiving material 1 could be obtained.

### (Preparation of a transferred image and the image evaluation)

The ink layers of the foregoing thermal-transfer materials A through J and the image-receiving layer of image-receiving material 1 were superposed together, respectively, and a thermal head was attached to the rear surface of each of the thermal-transfer materials. When an image was recorded thereon under the following conditions, each image having an excellent gradation was come out.

Heating time: Adjusted stepwise between 20 and 0.2msec.

The results of the evaluation of the images obtained are shown in Table 1.

### COMPARATIVE EXAMPLE 1

Comparative thermal-transfer materials K and L each having the same constitution as those of thermal-transfer materials Athrough C, except that the dye salts used in thermal-transfer materials Athrough C of Example 1 were replaced by dyes (1-1 through 3), independently. Images were each formed by making use of these materials in the same manner as in Example 1. Resultingly, any one of images having a clear hue could not be obtained, but they had also a maximum density lower than in the case of making use of the dye salts of the invention. In the comparative materials K and L, dye depositions were observed while preserving them. In the thermal-transfer materials of the invention, however, no dye deposition was observed at all.

### EXAMPLE 2

The surfaces of the foregoing thermal-transfer materials A through M and the rear surfaces of the same thermal-transfer materials were superposed each other, respectively. Each of the superposed matters was allowed to stand at 50°C for 48 hours and then the preservabilities of the thermal-transfer materials were each evaluated by observing the degrees of the bleeding-through of the dyes.

In the materials A through J of the invention, no bleeding-through of the dyes was observed at all. In the comparative materials K through M, however, the bleeding-through of the dyes were observed. In conclusion, the thermal-transfer materials of the invention were excellent in preservability and more improved in raw-stock preservability when further adding the base constituting a salt thereto.

### EXAMPLE 3

The following compound (ML-1) of 0.5 g/m² as a mordant was added to the image-receiving layer of image-receiving material 1 of Example 1, so that image-receiving material 2 was prepared. The following polymer mordant (ML-2) was added to image-receiving material 1 of Example 1, so that image-receiving material 2 was prepared.

An image was formed by making use of thermal-transfer material M having the same constitution as that of thermal-transfer material Aand in the combination of image-receiving materials 2 and 3. The maximum density and fixability of the resulting image are shown in Table 2. The fixability thereof were evaluated as follows.

### <Fixability>

The surface of the image-received layer was superposed on the coated surface of a sheet comprising a 5µm-thick polyester layer coated on a 180µm-thick polyethylene terephthalate film and they were heated at 140°C for minutes. The degrees of the dye-transfer to the polyester layer from the image-receiving layer were evaluated with the eye. It was proved that the less the re-transfers of the dyes were, the more the fixability was.
○ : No re-transfer was observed;
Δ : Slight re-transfers were observed; and
x : Remarkable re-transfers were observed.

In the case of the thermal-transfer material M, the transfer density and fixability were deteriorated (to be evaluated as Δ) when making use of image-receiving material 1.

### EXAMPLE 4

### (Synthesis of the chelate dye salt of the invention)

### CS-1 (Salt of dye C-1 and amine A-1)

C-1 (of 9.1 g) was suspended in ethyl acetate and A-1 (of 2.9 g) was then added thereto while stirring. After stirred at room temperature for 30 minutes, the resulting deposited crystals were filtrated. Yield : 9.2 g (79%); Melting point: 130 - 135°C.

### CS-2 (Salt of dye C-2 and amine A-1)

C-2 (of 12 g) was suspended in 500ml of ethyl acetate and A-1 (of 2.9 g) was then added thereto while stirring. After stirred at room temperature for 30 minutes, it was cooled down with ice and the resulting deposited crystals were filtrated. Yield : 5.8 g (38%)

### CS-3 (Salt of dye C-4 and amine A-19)

C-4 (of 15 g) was suspended in 300ml of acetone and A-19 (of 8.6 g) was then added thereto while stirring. After stirred at room temperature for 30 minutes, the resulting deposited crystals were filtrated. Yield : 8.4 g (36%)

### CS-4 (Salt of dye C-9 and amine A-1)

C-9 (of 6 g) was suspended in 50ml of ethyl acetate and A-1 (of 2.5 g) was then added thereto white stirring. After stirred at room temperature for 30 minutes, the resulting solids were filtrated. Yield : 4.6 g (52%)

### CS-5 (Salt of dye C-14 and amine A-1)

C-14 (of 11.32 g) was suspended in ethyl acetate and A-1 (of 2.9 g) was then added thereto while stirring. After stirred at room temperature for 30 minutes, the resulting crystals were filtrated. Yield : 10.6 g (72%)

### CS-6 (Salt of dye C-15 and amine A-1)

C-15 (of 8.9 g) was suspended in ethyl acetate and A-1 (of 2.8 g) was then added thereto while stirring. After stirred at room temperature for 30 minutes, the resulting crystals were filtrated. Yield : 9.5 g (81 %)

### CS-7 (Salt of dye C-1 and amine A-4)

C-1 (of 10.1 g) was suspended in 200ml of ethyl acetate and A-4 (of 5.8 g) was then added thereto while stirring. After heated at 50°C for 10 minutes, the solvent was distilled off and the resulting solids were filtrated. Yield : 15.6 g (98%)

### CS-8 (Salt of dye C-1 and amine A-14)

C-1 (of 8.1 g) was suspended in ethyl acetate and A-14 (of 2.4 g) was then added thereto while stirring. After stirred at room temperature for 30 minutes, the resulting crystals were filtrated. Yield : 9.6 g (91 %)

### CS-9 (Salt of dye M-2 and amine A-1)

M-2 (of 5 g) was suspended in 50ml of ethyl acetate and A-1 (of 1.3 g) was then added thereto while stirring. After heated at 50°C for 10 minutes, it became syrupy. Then, 50ml of acetone was added thereto and the resulting solids were filtrated. Yield : 4.3 g (57%)

### CS-10 (Salt of dye M-4 and amine A-1)

M-4 (of 3 g) was suspended in 50ml of ethyl acetate and A-1 (of 1.3 g) was then added thereto while stirring. When heated at 50°C for 10 minutes, it became syrupy. The resulting solids were filtrated. Yield : 3.5 g (82%)

The following syntheses were carried out in the same manner as in the above-described examples of the syntheses, so that the chelate dye salts were obtained.
CS-11 (Salt of dye M-6 and amine A-1)
CS-12 (Salt of dye M-8 and amine A-1)
CS-13 (Salt of dye M-8 and amine A-4)
CS-14 (Salt of dye Y-1 and amine A-1)
CS-15 (Salt of dye Y-4 and amine A-4)

### (Preparation of an ink)

A uniform ink solution containing a thermodiffusible dye was obtained from the mixture having the following composition.

### (Preparation of Thermal-transfer materials)

On a support comprising a 4.5µm-thick polyethylene terephthalate film, the above-mentioned ink was coated by a wire-bar and then dried so as to have a dried coating weight of 1.0 g/m², so that a layer containing a thermodiffusible dye could be formed and thereby thermal-transfer material 1 of the invention could be prepared. The rear surface of the polyethylene terephthalate film was provided thereon with a nitrocellulose layer containing silicone-denatured urethane resin (SP-2105 manufactured by Dai-Nichi Seika) for serving as a sticking preventive layer.

In the same manner as mentioned above, thermal-transfer materials 2 through 15 were each prepared, except that dye salt CS-1 was replaced by CS-2 through CS-15, respectively. Besides, comparative thermal-transfer materials 16 through 19 were also prepared in the same manner as in thermal-transfer material 1, except that dye salt CS-1 was replaced by independent dyes C-1, M-6 and Y-1 and comparative dye C-0 in an equivalent mol, respectively.

### (Preparation of Image-receiving material)

On a paper support laminated with polyethylene on the both surfaces thereof [which contained a suitable amount of a white pigment (Ti0₂), a bluish coloring agent and the following metal source (in a content of g/m2)], a vinyl chloride resin containing silicone oil (in a content of 0.15 g/m²) was coated as an image-receiving layer so as to have a coated weight of 10 g/m², so that an image-receiving material could be prepared.
Metal source : [Ni(NH₂COCH₂CH₂NHC₃H₇)₃]2⁺2[(C₆H₅)₄B⁻]

### (Formation of a transferred image and the image evaluation)

The coated surfaces of the resulting thermal-transfer recording materials 1 through 18 were superposed, respectively, face to face on the image-receiving layer of the image-receiving material. A thermal head was brought into contact with the thermal-transfer materials from the rear surface side, respectively, and then an image was recorded (under the same conditions as in Example 1).

An image-receiving material not containing any metal source was prepared in place of the above-described image-receiving material, and an image was recorded from the resulting image-receiving material and thermal-transfer recording material 19.

About each of the resulting images, the maximum reflection density (Dmax), the chelated reactivity of the dyes and the hue and fixability of the images were each evaluated according to the following criteria. The results thereof are shown in Table 3.

### <Fixability>

The imaged surface of the image-receiving layer was superposed on the coated surface of a transfer-sheet comprising a 5µm-thick nitrocellulose layer coated on a 180µm-thick polyethylene terephthalate film. The superposed layers were heated at 140°C for one minute, so that the degrees of dyes transferred from the image-receiving layer to the nitrocellulose layer were evaluated with the eye. It was proved thatthe less the re-transfer of the dyes was, the more the fixability was excellent.
○ : No re-transfer was observed;
Δ : Slight re-transfers were observed; and
x : Remarkable re-transfers were observed.

### <Hue>

○ : Satisfactory for the hues of cyan, magenta and yellow;
Δ : Unsatisfactory for the hues to some degree; and
x : Unsatisfactory for the hues

The light fastness is indicated by a dye residual ratio (%) obtained after exposing the images to a xenon fade-o-meter for 3 days; and the sensitivity was evaluated by the reflection density obtained when applying an energy of 6 msec.

The maximum reflection density (Dmax) was measured by means of an optical densitometer (Model PDA-65 manufactured by Konica Corp.)

As compared to the comparative samples, it was proved from Table 3 that every sample of the invention was high in sensitivity, excellent in fixability and rapid in chelating rate and, therefore, they had an excellent hue having few color contaminations, so that an excellent light fast image can be obtained.

As is proved by the above-given examples, a color image having an excellent hue and a high density can be obtained when making use of the thermal-transfer materials of the invention and, in addition, the fixability of the resulting image can also be excellent. The effects of the fixability can be more than in the case where a mordant is contained in an image-receiving material.

These effects can be displayed by making use of the salts of a dye having a phenolic hydroxyl group as the dye for forming an image and an organic base.

## Claims

1. A thermal-transfer material comprising a support having thereon a layer containing a dye, wherein said dye is a salt of a nitrogen-containing organic base.

2. The thermal-transfer material of claim 1 wherein said dye contains a phenolic hydroxy group.

3. The thermal-transfer material of claim 2 wherein said dye containing a phenolic hydroxy group is represented by formula I:
wherein R represents a group forming an azomethine dye together with =N-C₆H₄-OH, wherein the benzene ring may have a substituent.

4. The thermal-transfer material of claim 1 wherein said dye is a chelatable dye.

5. The material of claim 4 wherein said chelatable dye is a 3-coordinated chelatable dye.

6. The material of claim 5 wherein said 3-coordinated chelatable dye is represented by formula II:
wherein A represents an aryl group or a heterocyclic group in which at least one of the adjacent positions to the carbon atom being connected to the azo bond, is a carbon atom substituted with a chelatable group or a chelatable hetero atom; and Z represents a group consisting of atoms necessary to form a 5- or 6- membered ring.

7. The material of claim 1 wherein the nitrogen-containing organic base has a pKa of not less than 9.

8. The material of claim 7 wherein the base is represented by formula III,
wherein R₁, R₂ and R₃ represent each a hydrogen atom or an alkyl group; R₄ represents a hydrogen atom, an alkyl group, an aryl group, an amino group including an alkyl-substituted amino group or a guanidine group, provided R₁ and R₂, and R₃ and R₄, each may form a ring; X represents a vinyl group; and n is an integer of 0 or 1.

9. An image-forming process comprising: bringing a thermal-transfer material which contains a salt of a dye with a nitrogen-containing organic base on a support into contact with an image-receiving material having an image-receiving layer which contains a mordant containing a nitrogen-containing compound; applying heat on said thermal-transfer material in accordance with an image information; and forming an image in the image-receiving layer.

10. An image-forming process comprising; bringing a thermal-transfer material which contains a salt of a chelatable dye with a nitrogen-containing organic base on a support into contact with an image-receiving material having an image-receiving layer in the presence of a metal ion-supplying compound; applying heat on said thermal-transfer material in accordance with an image information; and forming an image in the image-receiving layer.
